

(No Model.)

L. L. SMITH.  
Coating Wire.

No. 241,741.

Patented May 17, 1881.

Fig. 1.



Fig. 2.



Fig. 3.



Witnesses:

M. L. Adams,  
as a Farr.

Inventor:  
L. L. Smith  
Per Edu. C. Quincy  
Atty.

# UNITED STATES PATENT OFFICE.

LUTHER L. SMITH, OF ANSONIA, CONNECTICUT.

## COATING WIRE.

SPECIFICATION forming part of Letters Patent No. 241,741, dated May 17, 1881.

Application filed March 9, 1881. (No model.)

*To all whom it may concern:*

Be it known that I, LUTHER L. SMITH, of Ansonia, Connecticut, have invented a Process for Effecting the Uniform Electro-Deposition 5 of Metal upon Wire, of which the following is a specification.

My invention is especially applicable to the purpose of covering iron and steel wire with an electro-deposit of copper.

It is the object of my invention to overcome that part of the difficulty in evenly coating wire by electro-deposition which arises from the variable energy with which different parts of the electrolytic solution act, in order that I 15 may be able to cover all parts of a coil or coils of wire of indefinite length with an electro-deposit of uniform thickness; and my invention consists in so manipulating a coil of wire of indefinite length—such, for instance, as a coil 20 of telegraph-wire as it comes from the manufacturer, or a series of coils joined end to end—that they are conducted progressively through the plating-solution in a helical path at a uniform rate of speed, which is regulated with reference to such prolongation of the exposure of 25 the wire to electrolytic action as may be necessary to produce a deposit of the desired thickness. Apparatus for economically accomplishing this result should have the capacity 30 to slightly separate the successive convolutions of the coil from each other, and to cause the coil to rotate upon its axis in a horizontal plane, while the convolutions of the coil are either wholly or partially submerged in the electrolytic solution. By this mode of manipulating 35 the wire all parts of the coil or coils are conducted progressively through the same parts of the electrolytic solution, and are subjected to like conditions of exposure to variations 40 which may exist in the relative energy with which the different parts of the solution act. It hence follows that the obtaining of a uniform coating upon all parts of any number of coils of wire requires only the exercise of ordinary care in regulating the strength of the 45 electric current employed and the area of the immersed anode surface.

As I have made the apparatus which I prefer to use in practicing my process the subject 50 of a separate application for a patent, I do not

base any claim upon it herein. The said apparatus is illustrated in the accompanying drawings, in which—

Figure 1 is a top view. Fig. 2 is a side elevation, partly in section; and Fig. 3, a transverse vertical section.

The apparatus consists of a tank, A, of suitable dimensions, on the top of which there is mounted a rotating shaft, B, for supporting the several convolutions of the coils of wire C. 60 The several convolutions of wire are kept separate from each other by the wooden racks D, which float upon the surface of the solution, in which are inserted the usual anodes, E. By the use of that apparatus wire hung upon a 65 horizontal rotating metallic impelling-roller is made a part of an electric circuit, which includes the electrolytic solution and the anodes therein immersed, and is introduced into and carried through and out of the solution in a 70 helical path at a rate of speed graduated at the will of the operator, according to the requirements of the case.

When a coil of wire in mass is immersed in a plating-solution it occasionally happens that 75 portions of the wire lying in a part of the solution where the electrolytic action is feeble are attacked by the acid in the solution before there is time for a sufficient electro-deposit upon them to protect them from the acid, and 80 the portions thus attacked may be thereby prevented from taking an electro-deposit. By my process the wire moves progressively, and is made to enter at the surface of the solution at a point where the electrolytic action is so 85 energetic that there is formed upon the surface of the wire, soon after it enters, an electro-deposit of sufficient thickness to protect the wire from the action of the acid in the solution. It is by this feature of my process, together with the subjection of all parts of the 90 wire progressively to like conditions or to a like series of variable conditions of electrolytic action that I am enabled to insure the production of a coil or coils of wire of indefinite length all parts of which are covered with 95 an electro-deposit of uniform thickness.

As will be seen, therefore, my process has two distinct characteristics: first, the progressive introduction of the wire into and its pas- 100

sage through and out of the electrolytic solution at a prescribed rate of speed, irrespectively of the form of the path of the wire in the solution; and, secondly, the conduct of the wire 5 progressively through the electrolytic solution in a helical path, whereby a large quantity of wire may be acted upon at the same time by an electrolytic solution contained in a tank of moderate dimensions.

- 10 I claim as my invention—  
The method herein described of covering with

a deposit of metal a coil of wire by causing it to revolve so that the wire will enter continuously at one place an electrolytic solution forming part of an electric circuit of which the 15 wire is an electrode, travel through it in a spiral course, and pass out at another place, receiving the deposit of metal in its course.

LUTHER L. SMITH.

Witnesses:

THOS. WALLACE,  
W. G. BENHAM.